

1,495,961

May 27, 1924.

M. H. NEWELL ET AL

PROCESS FOR THE PRODUCTION OF METAL POWDER OR DUST

Filed Feb. 15, 1923

2 Sheets-Sheet 1

Figure 1.



Figure 2.



INVENTORS

Minton H. Newell  
Evald Anderson

BY

Arthur P. Knights

ATTORNEY

May 27, 1924.

1,495,961

M. H. NEWELL ET AL

# PROCESS FOR THE PRODUCTION OF METAL POWDER OR DUST

Filed Feb. 15, 1923

Figure 3.



INVENTORS:  
*Minton H. Newell*  
*Evald Anderson*  
BY  
*Arthur P. Knight*  
ATTORNEY

## UNITED STATES PATENT OFFICE.

MINTON H. NEWELL, OF PALO ALTO, AND EVALD ANDERSON, OF ALHAMBRA, CALIFORNIA, ASSIGNORS TO INTERNATIONAL PRECIPITATION COMPANY, OF LOS ANGELES, CALIFORNIA, A CORPORATION OF CALIFORNIA.

## PROCESS FOR THE PRODUCTION OF METAL POWDER OR DUST.

Application filed February 15, 1923. Serial No. 619,324.

To all whom it may concern:

Be it known that we, MINTON H. NEWELL and EVALD ANDERSON, citizens of the United States, residing, respectively, at Palo Alto, in the county of Santa Clara, and at Alhambra, in the county of Los Angeles, State of California, have invented a new and useful Process for the Production of Metal Powder or Dust, of which the following is a specification.

This invention relates more especially to the production of finely divided zinc, zinc powder or dust, which is especially adapted for use as a precipitant in the recovery of gold, silver and other metals by the cyanide process and as a reducing agent in the dye industry, and for other purposes. The process may, however, be used for production of dust or powder of other metals.

The main object of the present invention is to provide for production of said zinc powder in a state of extremely fine division and having a high precipitating or reducing efficiency. Our invention consists essentially in producing zinc vapor by volatilization of metallic zinc or otherwise, bringing such zinc vapor, while still at high temperature into contact with a relatively cooler gaseous medium containing an oxidizing constituent, thereby causing condensation of the zinc in finely divided form and then separating the finely divided zinc so condensed from the gases. Our process also comprises circulation of the gases in such manner that the same gas is used rapidly in cyclic operation for cooling further quantities of zinc vapor to condense the same to finely divided zinc, definite and regulated quantity of oxidizing agent being supplied to the gases to maintain the required oxidizing property thereof. The accompanying drawings illustrate apparatus suitable for our invention and referring thereto Fig. 1 is a plan and Fig. 2 is a side elevation section of a preferred form of such apparatus, the retorting furnace being shown in section. Fig. 3 is a vertical section of a modified form thereof.

Referring to Fig. 2, we have indicated at 1 a zinc volatilizing retort provided with a suitable furnace means 2 for heating the same and with an outlet 3 discharging into a casing or chamber 4 which serves as a condensing and settling chamber, said chamber

being provided at its lower portion with a 55 suitable means such as a funnel or hopper 5, for receiving the zinc powder and with a gate or discharge means 6, whereby the settled powder may be withdrawn from time to time in a suitable receiving means. Said 60 chamber 4 is sealed by clay 14, or other suitable material so as to make an airtight joint between chamber 4 and furnace 2.

Means are provided for circulating the gas from the cooler part of the chamber 4 to the portion thereof adjacent to the mouth or outlet of the retort 1. For this purpose a fan or blower 7 may be provided, operated by suitable means and having its intake 8 connected to a portion of the chamber 4 removed from retort 1 and its outlet connected by a conduit 9 which discharges into the chamber 4 adjacent to said outlet 3 of the retort 1, or in position to direct current of gas therefrom into contact with the vapor 75 issuing from said outlet.

Means are also provided for a supply of definite and regulated amount of oxidizing agent to the chamber 4. For this purpose a so-called breathing bag indicated at 10 80 may be provided, communicating to an opening 11 with the chamber 4 and exposed to the outer air, said bag being of suitable permeable material such as cloth, so as to permit restricted communication of gases 85 therethrough, the amount of restriction depending on the closeness of weave of the cloth so that any desired amount of restriction can be secured by properly choosing a cloth of suitable texture. The wall of chamber 4 may be provided with an opening normally closed by plug 13 to serve as a sight opening and for the passage of a tool for cleaning the interior of the casing.

Our process may be carried out in the 95 above described apparatus as follows: Spelter, zinc dross or other material containing metallic zinc or zinc alloy, is introduced into the retort 1 and the latter is then heated so as to volatilize the zinc, the zinc vapor escaping through the outlet 3 into the chamber 4. Immediately on entering said chamber 4, the zinc vapor, while still at a high temperature is brought into contact with relatively cool gas discharged from the conduit 9, thereby chilling the zinc vapor and causing it to condense in the form of dust or powder. Assuming that the operation is 100 105

started with atmospheric air contained in the chamber 4, the effect of the oxidizing action of the air on the zinc vapor will be in the first instance to produce oxide of zinc, 5 but in continued operation of the process the gas within the chamber 4 eventually becomes deprived of oxygen to such an extent that only a relatively small proportion of oxygen remains and only a slight oxidizing 10 effect takes place on the zinc. The chamber 4 is of a relatively large capacity and has sufficiently large superficial area to provide for the required cooling of the gases contained therein so that the gas drawn from 15 the chamber at a point remote from the retort and then forced by the blower to a part adjacent to the retort, is sufficiently cool to produce the required condensing action on the zinc vapor. Sufficient air is continually 20 or intermittently supplied through the means 10 to maintain the proportion of oxygen in the gas in the chamber 4, required for most effective production of the finely divided zinc powder. We have found that for some 25 purposes it is desirable to maintain an oxygen content such that the resulting zinc dust contains not less than 84 per cent or more than 96 per cent metallic zinc.

In further explanation of the operation 30 of the so-called breathing bag 10, it may be stated that in the operation of the apparatus slight fluctuation of pressure results in chamber 4, probably due to intermittent supersaturation of the gases with zinc vapor, 35 followed by or alternating with periods of rapid condensation which are accompanied by corresponding degrees of pressure within the chamber and during such periods of decreased pressure a certain amount of atmospheric air will pass into the chamber, thereby introducing a fresh supply of oxygen. On the other hand, during periods 40 when the supersaturated condition is building up in the chamber, there is a corresponding increase of pressure during which a certain amount of gases will be expelled through the bag 10, said bag, however, preventing the outward passage of suspended zinc powder with such expelled gases.

50 We have found that both the chilling of the vapor produced by circulation of the gases as stated and the presence of a limited amount of oxidizing agent are necessary for the production of the most effective zinc dust for certain purposes; for example, as 55 a precipitant in the cyanide process of extraction of metals. In place of air, any oxidizing agents may be used, by which controlled partial oxidation of zinc vapor or 60 zinc dust can be carried on, for example, carbon dioxide, steam or other gas or vapor containing oxygen in combined form, but capable of producing an oxidizing action on zinc may be introduced into chamber 4, for 65 example, through a pipe or conduit 12.

Our process may also be carried out in any other suitable form of apparatus providing for the essential steps in the operation as above described, for example, in an apparatus such as shown in Fig. 3, the zinc 70 volatilizing retort 1 in that case discharging into a chamber or flue 4 leading to a filter apparatus such as bags 15 which are provided with suitable means for removing the collecting material therefrom in the usual 75 manner, such material being withdrawn through a gate means 6 and the gases being withdrawn from the bags through a conduit 16 by pump or blower 7 and forced back through a conduit 9 into proximity to the 80 outlet 3 of retort 1. In this case we have shown regulatable inlet means or valve 12 for admitting air or other oxidizing gas or vapor to the chamber 4 and the regulatable outlet means or valve 18 for discharging 85 gases from the circulating system in such manner as to maintain the required oxidizing property of the gases into contact with which the zinc vapor is introduced. Oxidizing gases may be introduced at valve 12 90 continuously or intermittently as may be required, or valves 12 and 18 may be closed and a bag 10 of suitable permeable material may be attached to an opening 11 communicating with chamber 4. The wall of chamber 4 may be provided with an opening normally closed by plug 13 to serve as a side opening and for passage of a tool for cleaning the interior of the casing.

What we claim is:

1. The process for producing metal dust or powder which consists in producing the vapor of the metal by action of heat on material containing such metal, bringing such vapor into contact with a gaseous medium which is at a sufficiently low temperature to cause condensation of the zinc vapor, such gaseous medium being capable of producing sufficient oxidation of the metal to insure condensation into finely divided solid particles, removing from the gaseous medium the solid metal particles suspended therein, cooling the gaseous medium and returning it to contact with fresh portions of metal vapor and maintaining a definite and regulated supply of oxidizing agent to the gaseous medium to maintain the oxidizing property thereof.

2. The process which consists in subjecting material containing zinc to heat to produce zinc vapor, introducing such vapor into a chamber, introducing into said chamber a relatively cool gaseous medium in such manner that the said medium is brought into contact with the zinc vapor and causes a condensation thereof, removing from the gases, the solid zinc particles produced therein, withdrawing a portion of the gases from said chamber and returning the portion so withdrawn and in relatively cool condition

to contact with fresh portions of zinc vapor introduced into the chamber and admitting to said chamber a definite regulated amount of oxidizing agent to maintain the said 5 gaseous medium in the chamber in oxidizing condition.

3. A process for production of metal dust or vapor comprising vaporizing metal, introducing the vapor into a gaseous medium 10 containing a limited regulated supply of oxygen and at a sufficiently low temperature to cause condensation of the vapor, subjecting such gaseous medium to cooling action, circulating such gaseous medium from a 15 cooler portion thereof to a portion thereof adjacent to the point of introduction of the metallic vapor to effect cooling and condensation of the metallic vapor.

4. A process for production of metal dust 20 or powder comprising vaporizing the metal and supplying to the vapor a limited

amount of gaseous medium containing a limited amount of an oxidizing agent, circulating said gaseous medium from cooler portions thereof to portions adjacent to the 25 point of contact with the metallic vapor so as to condense the vapor by contact with such cooler gaseous medium and collecting the condensed material.

5. A process for production of zinc dust 30 or powder comprising vaporizing the zinc, introducing the zinc vapor into a body of gaseous medium moving in a circulatory path, said gaseous medium containing a controlled amount of oxidizing agent and being 35 cooled in a portion of its path in such manner as to effect condensation of the zinc vapor when introduced thereinto and controlling the supply of oxidizing agent to said gaseous medium.

MINTON H. NEWELL.  
EVALD ANDERSON.